

No. 683,311.

Patented Sept. 24, 1901.

F. M. MARCY.

DRAWING ROLL.

(Application filed June 6, 1900.)

(No Model.)



Witnesses,  
Edward F. Allen.  
Thomas J. Drummond.

Entered by,  
Frank M. Marcy,  
by Crosby Gregory,  
attys.

# UNITED STATES PATENT OFFICE.

FRANK M. MARCY, OF WORCESTER, MASSACHUSETTS, ASSIGNOR OF ONE-HALF TO DRAPER COMPANY, OF PORTLAND, MAINE, AND HOPEDALE, MASSACHUSETTS.

## DRAWING-ROLL.

SPECIFICATION forming part of Letters Patent No. 683,811, dated September 24, 1901.

Application filed June 6, 1900. Serial No. 19,209. (No model.)

*To all whom it may concern:*

Be it known that I, FRANK M. MARCY, a citizen of the United States, residing at Worcester, county of Worcester, and State of Massachusetts, have invented an Improvement in Drawing-Rolls, of which the following description, in connection with the accompanying drawing, is a specification, like letters on the drawing representing like parts.

10 This invention relates to drawing-rolls for spinning-frames and the like, and more particularly to top rolls, which are usually made with a metal body and a covering of felt and leather. It is well known that these rolls 15 wear very rapidly, and the re-covering is a very large item of expense, and it is my object to avoid this expense and produce a roll having a very durable wearing-surface, yet the full equivalent, so far as efficiency is concerned, of the well-known leather-covered roll in first-class condition.

20 My invention comprises the roll and the process of treating the same to increase its wearing properties and life, and the process 25 is adapted to either new rolls or worn ones, although particularly adapted to the latter.

The drawing represents, in elevation and part section, a drawing-roll to clearly illustrate my invention.

30 The metal body *a* and leather cover *b* therefore are and may be of usual or well-known construction.

In carrying out my invention I coat the 35 leather cover with an enameling composition, which produces a fine wear-resisting surface and greatly enhances the life of the roll.

40 In conducting my experiments I have used a composition consisting of a viscous vehicle, a thickener, and a drier, and I have found that with boiled linseed-oil, lampblack, and japan, used as a vehicle, thickener, and drier, respectively, the following proportions produce good results: one-half pint boiled linseed-oil, lampblack enough to 45 give the consistency of thick cream thoroughly mixed with the oil, and three spoonfuls of japan or the same quantity of naphtha. The proportions above given may be varied according to circumstances.

50 The roll is placed in a naphtha solution to extract the oil or grease from the leather, and thereafter the enamel is applied.

Before applying the enamel I have found it desirable to apply shellac or the like to the roll, and for convenience the roll is placed on 55 an arbor and revolved in any suitable manner, shellac being applied by means of a piece of cloth pressed against the revolving surface of the roll, any rough places on the leather being thereby smoothed down and giving a 60 good even surface of the enamel. The enamel is then applied to the roll in any suitable or convenient manner, as by a brush or pad, to thoroughly impregnate the roll-cover, and thereafter the roll is baked for, say, two and 65 one-half hours at a temperature of about 150° Fahrenheit, and the covering *b* of the roll will present a fine, smooth, and durable coating or finish, (indicated at *c* in the drawing.)

70 My invention is not restricted to the precise proportions or manipulations herein set forth, and, so far as I am aware, it is broadly new to apply enamel to the cover of a drawing-roll.

Having described my invention, what I 75 claim as new, and desire to secure by Letters Patent, is—

1. As an article of manufacture, a drawing-roll having a leather cover provided with 80 an enamel finish.

2. As an article of manufacture, a drawing-roll having a leather cover shellacked and impregnated with an enamel composition.

3. As an article of manufacture, a leather-covered drawing-roll having an enamel composition baked thereon.

4. As an article of manufacture, a drawing-roll having a leather cover impregnated with a mixture of linseed-oil, lampblack and a drier, as japan.

5. The process of finishing leather-covered drawing-rolls which consists in applying to the leather an enamel, and baking the same.

6. The process of finishing leather-covered drawing-rolls which consists in applying shellac to the leather, coating with an enamel, and baking the same.

7. The process of finishing leather-covered drawing-rolls which consists in applying to the leather a composition containing a viscous vehicle, a thickener, and a drier, and thereafter subjecting the same to a baking temperature.

8. The process of finishing leather-covered

drawing-rolls which consists in removing the oil or grease from the leather, applying a composition of japan, lampblack and linseed-oil thereto, and thereafter baking the roll.

5 9. The process of finishing leather-covered drawing-rolls which consists in removing the oil or grease from the leather, applying a composition of japan lampblack and linseed-oil thereto, and thereafter subjecting the roll to

a baking temperature of substantially 150° to Fahrenheit.

In testimony whereof I have signed my name to this specification in the presence of two subscribing witnesses.

FRANK M. MARCY.

Witnesses:

H. N. PARKER,  
A. R. BRIGHAM.